

Oct. 29, 1957

R. W. FRITTS ET AL  
ELECTRICALLY CONDUCTIVE COMPOSITIONS  
AND METHOD OF MANUFACTURE THEREOF

2,811,721

Filed Dec. 15, 1954

4 Sheets-Sheet 1

Fig. 2.



Fig. 1.



Fig. 1.

INVENTORS  
Robert W. Fritts,  
BY Sebastian Karrer,  
Brown, Boveri, Büttda & Cie  
Atty's  
S.

Oct. 29, 1957

R. W. FRITTS ET AL  
ELECTRICALLY CONDUCTIVE COMPOSITIONS  
AND METHOD OF MANUFACTURE THEREOF

2,811,721

Filed Dec. 15, 1954

4 Sheets-Sheet 2



INVENTORS  
Robert W. Fritts

BY Sebastian Karrer,

Orman, Johnson, Baetke & Oliver

Atty S.

Oct. 29, 1957

R. W. FRITTS ET AL  
ELECTRICALLY CONDUCTIVE COMPOSITIONS  
AND METHOD OF MANUFACTURE THEREOF

2,811,721

Filed Dec. 15, 1954

4 Sheets-Sheet 3

ROOM TEMPERATURE  
THERMOELECTRIC POWER-MICROVOLTS/°C.



Fig. 4A.

300

ROOM TEMPERATURE  
THERMOELECTRIC POWER  
MICROVOLTS/°C.



0.001 .001 .01 .10 1.0  
WEIGHT PERCENT NEGATIVE PROMOTER - LOG SCALE

INVENTORS  
Robert W. Fritts,  
BY Sebastian Karrer,

Attest:  
John F. Fritts, Sr.  
Attest:

Oct. 29, 1957

R. W. FRITTS ET AL  
ELECTRICALLY CONDUCTIVE COMPOSITIONS  
AND METHOD OF MANUFACTURE THEREOF

2,811,721

Filed Dec. 15, 1954

4 Sheets-Sheet 4



INVENTORS:  
Robert W. Fritts,  
BY Sebastian Karrer,

Attest:  
John H. Hallinan  
Attest:  
John H. Hallinan

1

2,811,721

**ELECTRICALLY CONDUCTIVE COMPOSITIONS  
AND METHOD OF MANUFACTURE THEREOF**

Robert W. Fritts, Elm Grove, Wis., and Sebastian Karrer, Port Republic, Md., assignors to Baso Inc., a corporation of Wisconsin

Application December 15, 1954, Serial No. 475,543

21 Claims. (Cl. 75—166)

This invention relates to semi-metallic alloys or compositions, composed in the main of lead and sulphur, and more particularly to electrical conductors comprising such alloys or compositions.

It is an object of the invention to provide electrically conductive alloys or compositions as aforesaid having now relationships of certain electrical characteristics.

A further object is to provide electrically conductive alloys or compositions of the character indicated, in which the magnitudes of certain of the electrical characteristics thereof are reproducible within desired ranges therefor.

A further object is to provide electrically conductive alloys or compositions of the character indicated, the electrical conductivity of which may be either positive or negative, as desired.

Another object is to provide electrically conductive alloys or compositions of the character indicated, the resistivity of which may be controlled in magnitude as desired.

A further object is to provide electrically conductive alloys or compositions as aforementioned, the electrical characteristics, particularly with respect to polarity, of which are controllable and reproducible.

A further object of the invention is to provide electrically conductive alloys or compositions as aforementioned, in which desired resistivities therefor are reproducible.

Another object is to provide electrically conductive alloys or compositions of the character indicated, the thermo-electric power of which may be controlled in magnitude as desired.

A further object is to provide electrically conductive alloys or compositions as aforementioned in which the polarity of thermoelectric power may be either positive or negative as desired.

A further object is to provide electrically conductive alloys or compositions as aforementioned, having new relationships of thermoelectric power and resistivity, and which are readily reproducible within desired ranges of such relationships.

A further object is to provide electrically conductive alloys or compositions, the electrical characteristics of which are substantially independent of prior heat treatment.

A further object of the invention concerns a method of fabrication of the aforementioned alloys or compositions to provide for the reproducible production thereof within desired ranges of thermoelectric power and resistivity.

A further object is to provide a method as last mentioned for arbitrarily rendering such alloys or compositions either of positive or negative polarity.

A further object is to provide alloys or compositions as aforementioned having adequate mechanical strength for practical applications over a wide temperature range.

A further object is to provide electrically conductive

2

alloys or compositions of the character above-mentioned which are chemically stable over a wide temperature range when shielded from oxidizing atmospheres.

A further object is to provide electrical conductors composed of the alloys or compositions of the present invention.

Now, in order to acquaint those skilled in the art with the manner of practicing and utilizing the present invention, there is hereinafter disclosed certain preferred embodiments of the invention.

In the drawings:

Figure 1 is a graphic illustration generally indicating the effect of various concentrations of negative and positive promoters with respect to the resistivity characteristics of the electrically conductive semi-metallic alloys or compositions of the invention;

Figure 2 is a graphic illustration generally indicating the effect of various concentrations of negative and positive promoters with respect to the thermoelectric power characteristics of the electrically conductive semi-metallic alloys or compositions of the invention;

Figures 3 and 3A are graphic illustrations of the resistivity characteristics of certain of the electrically conductive semi-metallic alloys or compositions of the invention, within certain ranges of additions of negative promoters therein;

Figures 4 and 4A are graphic illustrations of the thermoelectric power characteristics of the electrically conductive semi-metallic alloys or compositions depicted in Figures 3 and 3A, respectively;

Figure 5 is a graphic illustration of the resistivity characteristics of certain of the electrically conductive semi-metallic alloys or compositions of the invention, within certain ranges of additions of positive promoters therein; and

Figure 6 is a graphic illustration of the thermoelectric power characteristics of the electrically conductive semi-metallic alloys or compositions depicted in Figure 5.

The invention described and claimed herein utilizes a lead-sulphur base composition or alloy consisting essentially of lead in the range of 86.63% to 87.10% by weight, balance substantially all sulphur, and which base composition contains not more than 0.001% by weight of other matter.

Lead-sulphur base alloys within the aforementioned range and of the aforementioned purity are negative electrical conductors and exhibit high negative thermoelectric power, nominally higher electrical resistivity, and low thermal conductivity with respect to a metal. Such compositions or alloys have utility as electrical conductors.

In lead-sulphur base alloys of the aforementioned range and purity the magnitudes of the thermoelectric power and electrical resistivity are strongly dependent upon the heat treatment afforded the alloy during fabrication, thereby affording control of such properties by the heat treatment.

The aforementioned lead-sulphur alloys may be best described metallographically as two-phase alloys. It has been observed that these alloys, when sectioned and examined microscopically, comprise a major phase comprising crystal grains varying usually from 1 to 10 millimeters in size and between such grains there exist thin relatively darker regions of a second phase. The grains of the primary phase are crystals of the intermetallic compound lead-sulphide which contain approximately 86.60% lead by weight. The darker second phase, clearly discernible at the grain boundaries, is lead containing a minor concentration of sulphur.

The function of the second phase in such alloys is

thought to be threefold. First, the thermal equilibrium between the two phases, which is established by the heat treatment aforementioned, induces negative thermoelectric power and conductivity in the primary lead-sulphide phase which, because of its high concentration in the alloy, controls the electrical properties of the two-phase alloy. Secondly, the thin layers act as a cementing agent for the grains of the primary phase, thereby improving the mechanical strength of the alloy when compared to that of the pure intermetallic compound. This cementing action of the second phase improves the strength of an alloy in tension and compression at all temperatures up to 815° C. Thirdly, the second phase affords good electrical continuity in the polycrystalline alloy by rendering the intergranular component of electrical resistivity negligible. We have found that the actual concentration of second phase is not critical so long as the composition is maintained within the aforementioned specified ranges.

Lead-sulphur alloys containing less than 86.63% lead by weight do not usually exhibit reproducible physical and electrical properties when in a polycrystalline state, and in alloys containing more than 87.10% lead by weight the second phase regions are of such dimension that the electrical conductivity along the grain boundaries of the alloy cannot be neglected when compared with the conductivity through the primary phase. Moreover, unless the specified ranges of compositions and purity are adhered to, third element addition "promoters" hereinafter described will be rendered ineffective. Additionally, alloys having large concentrations of the aforementioned second phase are subject to plastic flow at high temperatures and for this further reason are not desirable for high temperature applications. Accordingly, the specified composition ranges and purity are to be considered critical.

It will be observed that since the electrical properties of the aforementioned alloys or compositions are dependent upon the equilibrium temperature from which they have been quenched, use of such alloys or compositions is limited to such temperatures as will not affect the electrical characteristics established by the quenching treatment. Accordingly, for high temperature applications requiring fixed values of electrical characteristics arbitrary changes in these characteristics must be derived from the adjustment of factors other than temperature and annealing history.

We have further discovered that the electrical characteristics of lead-sulphur base alloys or compositions of the aforementioned range and purity can be markedly and advantageously altered in a reproducible manner by the addition thereto of controlled amounts of matter other than lead or sulphur. For convenience, these additions are herein designated "third element additions" to distinguish them from the lead and sulphur constituents of the alloys of the invention.

The "third element additions" which we have found effective for the purposes of the present invention when added in minor amounts to the lead-sulphur base alloy aforementioned are: Zirconium, indium, bromine, chlorine, titanium, iodine, tantalum, bismuth, antimony, gallium, columbium, uranium, sodium, potassium, rubidium and silver.

The third element additions aforementioned may be either "positive promoters" or "negative promoters" as hereinafter defined, and the resultant alloy or composition may be a "positive" or "negative" alloy or composition or conductor, as also hereinafter defined.

A "negative" composition or alloy and a "negative" conductor is to be understood through this specification and appended claims as meaning an alloy, composition or conductor which exhibits negative conductivity as evidenced by Hall effect measurements or thermoelectric effect measurements, both taken at room temperature. Similarly, a "positive" composition or alloy and a "posi-

tive" conductor is to be understood as meaning an alloy, composition or conductor which exhibits positive conductivity as evidenced by Hall effect measurements or thermoelectric effect measurements, both taken at room temperature.

"Negative promoters" are those which, when added to the lead-sulphur base alloy previously defined, alter the electrical conductivity without changing the polarity of the conductivity or thermoelectric power of the base alloy (it being negative according to the preceding definition). "Positive promoters" are those which, when added to the lead-sulphur base alloy, cause at first, with very small additions, reduction in the conductivity of the alloy to a minimum value beyond which further increase in the concentration of the positive promoter causes an increase in the conductivity of the alloy accompanied by a reversal in the polarity of the conductivity and thermoelectric power, i. e., from negative to positive.

The functions of such negative and positive promoters should be contrasted for sake of clarity as follows:

(1) Increasing concentrations of the negative promoter elements cause increases in the conductivity and decrease of the thermoelectric power of the resulting alloy, as compared to that of the lead-sulphur base alloy, while preserving the negative polarity of the conductivity and thermoelectric power thereof.

(2) Increasing concentrations of positive promoter elements cause initially reductions in the conductivity and increase in the thermoelectric power of the lead-sulphur base alloy, until a minimum conductivity is reached whereupon the thermoelectric power and conductivity reverse polarity to the positive sense, and further increase in the concentrations of the positive promoter causes increase in the conductivity and decrease of the thermoelectric power in the resulting alloy.

The aforeindicated effects are graphically illustrated in Figures 1 and 2, wherein the effect of varying the concentrations of the aforementioned negative and positive promoters are plotted. In both Figures 1 and 2, the central vertical axes give the properties of the aforescribed base lead-sulphur alloy or composition. The left halves of each of the figures characterize the change, at room temperature, of the electrical properties of the lead-sulphur base alloys or compositions with the addition of the aforementioned negative promoters. It will be observed that the two drawings, Figures 1 and 2, have no scales applied thereto since the concentration ranges differ for each of the third element additions to be hereinafter described due to variations in atomic weights and concentration limits. The right halves of each of Figures 1 and 2 show the changes in the electrical properties as positive promoters are added to the base alloy or composition. It should be noted that for a given promoter element the maximum resistivity and the polarity reversal of the thermoelectric power occur at the same concentration. This concentration is indicated by "a" in Figures 1 and 2.

Table I below, first column thereof, lists certain elements which we have found effective as negative promoters when added to the aforementioned lead-sulphur base alloys or compositions. Second column of Table I lists the order of the maximum concentration limits by weight percent of such promoters to the base alloy effective for achieving the objects of the invention. It is to be understood that these concentration limits are the maximum which effectively alter the electrical properties of the base alloy. Concentrations in excess of the stated amounts of such additives have no appreciable effect in beneficially altering the electrical properties with which this invention is concerned, and in this sense the limits indicated are to be considered critical. The third and fourth columns of Table I set forth the electrical properties at room temperature of lead-sulphur alloys promoted with the maximum useful concentrations of the negative promoters, after high temperature annealing as hereinafter disclosed.

| Negative Promoters | Order of Maximum Effective Concentration Limits By Weight Percent | Thermoelectric Power, Micro-volts/ $^{\circ}$ C. | Resistivity, Ohm-Cm. |
|--------------------|-------------------------------------------------------------------|--------------------------------------------------|----------------------|
| Zirconium          | 0.40                                                              | -36                                              | 0.0022               |
| Indium             | 0.50                                                              | -54                                              | 0.0024               |
| Bromine            | 0.35                                                              | -54                                              | 0.0024               |
| Chlorine           | 0.15                                                              | -54                                              | 0.0025               |
| Titanium           | 0.20                                                              | -68                                              | 0.0029               |
| Iodine             | 0.55                                                              | -99                                              | 0.0042               |
| Tantalum           | 0.70                                                              | -99                                              | 0.0042               |
| Bismuth            | 11.0-3.0                                                          | -118                                             | 0.0061               |
| Antimony           | 1.0-3.0                                                           | -126                                             | 0.0064               |
| Gallium            | 0.30                                                              | -117                                             | 0.0058               |
| Columbium          | 0.40                                                              | -108                                             | 0.0023               |
| Uraniun            | 1.0                                                               | -99                                              | 0.0034               |

Figures 3, 3A, 4 and 4A of the drawings may be here referred to for a graphic illustration of the effect of the additions of the negative promoters of Table I with respect to the resistivity and thermoelectric power characteristics (measured at room temperature) afforded by addition to the lead-sulphur base alloys or compositions of each of the negative promoters set forth in Table I, and with the variations indicated in the amount thereof added in each case.

As previously mentioned, certain positive promoters may also be alloyed with the aforementioned lead-sulphur alloys, and such promoters are listed in column 1 of Table II below. The second column of Table II, like the corresponding column of Table I, sets forth the order of the maximum concentration limits by weight percent of such promoters to the base alloy effective for achieving the objects of the invention. Again, it will be observed that concentrations of the positive promoters to the lead-sulphur base alloy in amounts in excess of that contained in column 2 of Table II have no appreciable effect in beneficially altering the electrical properties with which this invention is concerned and in this sense the limits indicated are to be considered critical.

Column 3 of Table II sets forth the concentration by weight percent of the positive promoters listed at which the polarity of conductivity and thermoelectric power of the promoted alloy reverses. These are the concentration values for the promoters respectively, indicated generally by point "a" in Figures 1 and 2.

Columns 4 and 5 set forth the thermoelectric power and resistivity characteristics at room temperature of the alloy or composition resulting from the addition of the aforementioned positive promoters in the amount shown in column 2 after high temperature annealing and subsequent slow cooling as hereinafter disclosed.

Table II

| Positive Promoters | Order of Maximum Effective Concentration Limits By Weight Percent | Concentration, Weight Percent at Which Polarity Reverses (Point "a" Figures 1 and 2) | Thermoelectric Power, Micro-volts/ $^{\circ}$ C. | Resistivity, Ohm-Cm. |
|--------------------|-------------------------------------------------------------------|--------------------------------------------------------------------------------------|--------------------------------------------------|----------------------|
| Sodium             | 0.20                                                              | 0.02                                                                                 | +364                                             | 0.24                 |
| Potassium          | 0.30                                                              | 0.04                                                                                 | +446                                             | 0.32                 |
| Rubidium           | 0.70                                                              | 0.20                                                                                 | +450                                             | 0.20                 |
| Silver             | 2.0                                                               | 0.30                                                                                 | +270                                             | 0.02                 |

As aforementioned, the lead-sulphur base alloy previously described is a two-phase alloy. When the aforementioned third element additions are incorporated in the base alloy, such third element additions become distributed between the two phases. We have discovered that the nature of such distribution has negligible effect upon the electrical properties of the composition in all cases except that of bismuth and antimony. Accordingly, in the case of bismuth and antimony, the maximum effective concentration is dependent upon the lead content

of the lead-sulphur base alloy within the ranges stated therefor in Tables I and II. We have found 3.0% by weight bismuth to be the maximum effective concentration for lead-sulphur base alloys containing 87.10% lead; for base alloys containing less lead the maximum effective bismuth concentration is somewhat less, that is ranges down to 1.0% by weight when the lead content ranges down to 86.63%. Similarly, in the case of antimony, the maximum effective concentration is dependent upon the lead content of the lead-sulphur base alloy within the range stated therefor. We have found 3.0% by weight antimony to be the maximum effective concentration for lead-sulphur base alloys containing 87.10% lead; for base alloys containing less lead the maximum effective antimony concentration is somewhat less, that is ranges down to 0.50% by weight when the lead content ranges down to 86.63%. This behavior of bismuth and antimony is thought to be due to the formation of a bismuth-lead-sulphur or an antimony-lead-sulphur complex within the intergranular phase aforementioned which accounts for a portion of the addition. All other third element additions aforementioned, both positive and negative, form complexes with the second or intergranular phase aforementioned to a much lesser extent than do bismuth and antimony, and for purposes of this invention, in the cases of such other additions these effects are inconsequential. Accordingly, no changes in the concentration limits thereof are necessary as the proportions of lead and sulphur in the base alloy vary within the range stated therefor.

In Tables I and II above, the thermoelectric power and resistivity data given is in both cases for the 86.63% lead, balance substantially all sulphur composition containing the third element addition in question in the amount indicated in the table (in the case of bismuth and antimony, the lower maximum effective amount indicated).

Figures 5 and 6 of the drawings may be here referred to for a graphic illustration of the effect of the additions of the positive promoters of Table II with respect to the resistivity and thermoelectric power characteristics (measured at room temperature) afforded by addition to the lead-sulphur base alloys or compositions of each of the positive promoters set forth in Table II, and with the variations indicated in the amount thereof added in each case.

In connection with the aforementioned Figures 3 to 6, the logarithm of the percent by weight concentration, and the logarithm of the resistivity have been plotted for convenience, as will be understood by those skilled in the art, while thermoelectric power has been plotted linearly.

It will be observed upon examination of the data recorded in Figures 1 through 6, that a wide range of electrical properties can be induced in lead-sulphur base alloys by third element additions, either positive or negative as desired. Indium additions, for example, can reduce the resistivity of the lead-sulphur base alloy by more than a factor of approximately 20 while reducing the thermoelectric power by a factor of 5.

The aforementioned alloys or compositions and electrical conductors comprising the invention may be fabricated by melting together the alloy constituents aforementioned, within the concentration limits aforementioned. It is to be understood, however, that as has been previously indicated, the lead-sulphur alloys of the invention must be of a high order of purity, i. e., containing not in excess of the order of 0.001% by weight impurity. Such purity has been found to be necessary in practicing the present invention if the electrical properties of the alloys of this invention are to be reproducible. It is to be understood, however, that tellurium and selenium, because of their chemical similarity to and natural occurrence with sulphur, are frequently contaminants in commercial sulphur and are difficult and expensive to remove to the extent of purity as specified above. We have

found, however, that tellurium and selenium concentrations of the order usually found in commercially pure sulphur, usually less than 1%, cause no significant changes in the electrical properties of the alloys of this invention.

In the production of the new alloys or compositions of our invention and electrical conductors comprising the same, the constituents are melted at from 1115° C. to 1200° C. under a reducing atmosphere, and agitated to insure uniform distribution. The alloy may then be cast, formed or machined as desired. It is then preferably annealed to insure normalization of the alloy or composition. Such annealing may be accomplished at temperatures ranging from 540° C. to 815° C. for from 10 to 20 hours, the lesser time being required at the higher temperature. The aforementioned annealing may be conveniently accomplished by sealing the ingots of the alloy or composition within a quartz or Vycor envelope under an inert atmosphere. This prevents loss of material and hence preservation of the ingots during annealing and affords a simple method of handling. The aforescribed third element addition promoted compositions may then be slowly cooled to room temperature or quenched directly or at any intermediate temperature in cold water without substantially affecting the reproducibility of the desired electrical characteristics, especially as the concentration of the third element addition approaches its maximum effective concentration limit aforesaid. Thus, the heat treatment history of the alloy or composition becomes of lesser importance in the third element addition promoted compositions aforescribed as the concentration of the third element addition approaches the maximum effective limit aforesaid.

The third element promoted alloy or composition is a two-phase alloy having improved electrical properties as compared to the corresponding properties of the lead-sulphur base alloy. For example, the electrical properties of the third element addition promoted alloys or compositions are governed to a lesser extent by the heat treatment given the alloy, with variations in electrical properties considerably less than the variations exhibited by the lead-sulphur base alloy to which no third element has been added. Thus, the third element additions, in effect, reduce the dependency of the electrical properties upon prior heat treatment and in this sense tend to stabilize these properties to a higher degree than that achieved in the lead-sulphur base alloy. It may be stated as a general observation that the degree of stabilization increases with the concentration of the aforementioned third element additions up to the maximum effective amount thereof as above set forth. This lesser dependency of third element addition promoted alloys or compositions aforescribed and of electrical conductors comprising the same, markedly increases the utility thereof for high temperature applications. In this connection, however, where alloys including positive promoters are concerned and where the application temperature approaches 570° C. concentrations of the positive promoter approaching the maximum effective limit aforesaid should be used to insure maintenance of positive polarity of the composition.

Compositions of the present invention also exhibit the desired physical properties aforesaid. More specifically, they are mechanically strong and stable under operating conditions. The coefficient of thermal expansion is of the order of  $20 \times 10^{-6}/^{\circ}\text{C}$ .

We claim:

1. A composition consisting essentially of a base constituent consisting essentially of lead and sulphur, the percent by weight of lead being 86.63% to 87.10%, balance substantially all sulphur, and no more than of the order of 0.001% by weight of other matter except for a promoter selected from the group consisting of zirconium, indium, bromine, chlorine, titanium, iodine, tantalum, bismuth, antimony, gallium, columbium, uranium, so-

dium, potassium, rubidium and silver in an amount effective to modify the conductivity of said base constituent not in excess by weight percent of the lead and sulphur of said promoters as follows: 0.40 zirconium; 0.50 indium; 0.35 bromine; 0.15 chlorine; 0.20 titanium; 0.55 iodine; 0.70 tantalum; 0.30 gallium; 0.40 columbium; 1.0 uranium; 0.20 sodium; 0.30 potassium; 0.70 rubidium; 2.0 silver; and bismuth and antimony not in excess of from 1.0 to 3.0 and from 0.50 to 3.0, respectively, over the aforementioned range of lead.

5 2. A negative electrical conductor consisting essentially of a base constituent consisting essentially of 86.63% to 87.10% lead by weight, balance substantially all sulphur, and not more than of the order of 0.001% by weight of other material except for a member selected from the group consisting of zirconium, indium, bromine, chlorine, titanium, iodine, tantalum, bismuth, antimony, gallium, columbium, uranium, sodium, potassium, rubidium and silver, with the zirconium, indium, bromine, chlorine, 15 titanium, iodine, tantalum, bismuth, antimony, gallium, columbium, uranium, sodium, potassium, rubidium and silver, in an amount effective to modify the conductivity of said base constituent not in excess by weight percent of the lead and sulphur of said members as follows: 0.40 20 zirconium; 0.50 indium; 0.35 bromine; 0.15 chlorine; 0.20 titanium; 0.55 iodine; 0.70 tantalum; 0.30 gallium; 0.40 columbium; 1.0 uranium; 0.02 sodium; 0.04 potassium; 0.20 rubidium; 0.30 silver; and bismuth and antimony not 25 in excess of from 1.0 to 3.0 and from 0.50 to 3.0, respectively, over the aforementioned range of lead.

30 3. A composition consisting essentially of a lead-sulphur base constituent consisting essentially of from 86.63% to 87.10% by weight lead, the balance substantially all sulphur, and a member selected from the group 35 consisting of zirconium, indium, bromine, chlorine, titanium, iodine, tantalum, bismuth, antimony, gallium, columbium, uranium, sodium, potassium, rubidium and silver, in an amount effective to modify the conductivity of 40 said base constituent not in excess by weight percent of the lead and sulphur of said members as follows: 0.40 zirconium; 0.50 indium; 0.35 bromine; 0.15 chlorine; 0.20 titanium; 0.55 iodine; 0.70 tantalum; 0.30 gallium; 0.40 columbium; 1.0 uranium; 0.20 sodium; 0.30 potassium; 0.70 rubidium; 2.0 silver; and bismuth and antimony not 45 in excess of from 1.0 to 3.0 and from 0.50 to 3.0, respectively, over the aforementioned range of lead.

4. A composition consisting essentially of a lead-sulphur base constituent consisting essentially of from 86.63% to 87.10% lead by weight, balance substantially 50 all sulphur, and zirconium in an amount effective to modify the conductivity of said base constituent not in excess of 0.40% by weight of the lead and sulphur.

55 5. A composition consisting essentially of a lead-sulphur base constituent consisting essentially of from 86.63% to 87.10% lead by weight, balance substantially all sulphur, and indium in an amount effective to modify the conductivity of said base constituent not in excess of 0.50% by weight of the lead and sulphur.

60 6. A composition consisting essentially of a lead-sulphur base constituent consisting essentially of from 86.63% to 87.10% lead by weight, balance substantially all sulphur, and bromine in an amount effective to modify the conductivity of said base constituent not in excess of 0.35% by weight of the lead and sulphur.

65 7. A composition consisting essentially of a lead-sulphur base constituent consisting essentially of from 86.63% to 87.10% lead by weight, balance substantially all sulphur, and chlorine in an amount effective to modify the conductivity of said base constituent not in excess of 0.15% by weight of the lead and sulphur.

70 8. A composition consisting essentially of a lead-sulphur base constituent consisting essentially of from 86.63% to 87.10% lead by weight, balance substantially all sulphur, and titanium in an amount effective to modify

the conductivity of said base constituent not in excess of 0.20% by weight of the lead and sulphur.

9. A composition consisting essentially of a lead-sulphur base constituent consisting essentially of from 86.63% to 87.10% lead by weight, balance substantially all sulphur, and iodine in an amount effective to modify the conductivity of said base constituent not in excess of 0.55% by weight of the lead and sulphur.

10. A composition consisting essentially of a lead-sulphur base constituent consisting essentially of from 86.63% to 87.10% lead by weight, balance substantially all sulphur, and tantalum in an amount effective to modify the conductivity of said base constituent not in excess of 0.70% by weight of the lead and sulphur.

11. A composition consisting essentially of a lead-sulphur base constituent consisting essentially of from 86.63% to 87.10% lead by weight, balance substantially all sulphur, and bismuth in an amount effective to modify the conductivity of said base constituent not in excess of from 1.0% to 3.0% by weight of the lead and sulphur over the aforementioned range of lead.

12. A composition consisting essentially of a lead-sulphur base constituent consisting essentially of from 86.63% to 87.10% lead by weight, balance substantially all sulphur, and antimony in an amount effective to modify the conductivity of said base constituent not in excess of from 0.50% to 3.0% by weight of the lead and sulphur over the aforementioned range of lead.

13. A composition consisting essentially of a lead-sulphur base constituent consisting essentially of from 86.63% to 87.10% lead by weight, balance substantially all sulphur, and gallium in an amount effective to modify the conductivity of said base constituent not in excess of 0.30% by weight of the lead and sulphur.

14. A composition consisting essentially of a lead-sulphur base constituent consisting essentially of from 86.63% to 87.10% lead by weight, balance substantially all sulphur, and columbium in an amount effective to modify the conductivity of said base constituent not in excess of 0.40% by weight of the lead and sulphur.

15. A composition consisting essentially of a lead-sulphur base constituent consisting essentially of from 86.63% to 87.10% lead by weight, balance substantially all sulphur, and uranium in an amount effective to modify the conductivity of said base constituent not in excess of 1.0% by weight of the lead and sulphur.

16. A composition consisting essentially of a lead-sulphur base constituent consisting essentially of from 86.63% to 87.10% lead by weight, balance substantially all sulphur, and sodium in an amount effective to modify the conductivity of said base constituent not in excess of 0.20% by weight of the lead and sulphur.

17. A composition consisting essentially of a lead-sulphur base constituent consisting essentially of from 86.63% to 87.10% lead by weight, balance substantially all sulphur, and potassium in an amount effective to modify the conductivity of said base constituent not in excess of 0.30% by weight of the lead and sulphur.

18. A composition consisting essentially of a lead-sulphur base constituent consisting essentially of from 86.63% to 87.10% lead by weight, balance substantially all sulphur, and rubidium in an amount effective to modify the conductivity of said base constituent not in excess of 0.70% by weight of the lead and sulphur.

19. A composition consisting essentially of a lead-sulphur base constituent consisting essentially of from 86.63% to 87.10% lead by weight, balance substantially all sulphur, and silver in an amount effective to modify the conductivity of said base constituent not in excess of 2.0% by weight of the lead and sulphur.

20. The method of controlling the electrical characteristics of a lead-sulphur composition consisting essentially of from 86.63% to 87.10% lead by weight, balance substantially all sulphur, which comprises alloying therewith at least one member from the group consisting of zirconium, indium, bromine, chlorine, titanium, iodine, tantalum, bismuth, antimony, gallium, columbium, uranium, sodium, potassium, rubidium, and silver, in an amount not in excess by weight percent of the lead and sulphur of said members as follows: 0.40 zirconium; 0.50 indium; 0.35 bromine; 0.15 chlorine; 0.20 titanium; 0.55 iodine; 0.70 tantalum; 0.30 gallium; 0.04 columbium; 1.0 uranium; 0.20 sodium; 0.30 potassium; 0.70 rubidium; 2.0 silver; and bismuth and antimony not in excess of from 1.0% to 3.0% and from 0.50% to 3.0% respectively, over the aforesaid range of lead, and then annealing the resultant composition at a temperature of from about 30 540° C. to 815° C.

21. A multi-phase alloy consisting essentially of a base constituent consisting essentially of lead and sulphur, the percent by weight of lead being 86.63% to 87.10%, balance substantially all sulphur, having a phase constituting primarily the intermetallic compound lead-sulphide and having another phase constituting primarily excess lead, and no more than of the order of 0.001% by weight of other matter, except for a promoter selected from the group consisting of zirconium, indium, bromine, chlorine, titanium, iodine, tantalum, bismuth, antimony, gallium, columbium, uranium, sodium, potassium, rubidium and silver in an amount effective to modify the conductivity of the base constituent not in excess by weight percent of the lead and sulphur of said promoters as follows: 0.40 zirconium; 0.50 indium; 0.35 bromine; 0.15 chlorine; 0.20 titanium; 0.55 iodine; 0.70 tantalum; 0.30 gallium; 0.40 columbium; 1.0 uranium; 0.20 sodium; 0.30 potassium; 0.70 rubidium; 2.0 silver; and bismuth and antimony not in excess of from 1.0 to 3.0 and from 0.50 to 3.0, respectively, over the aforementioned range of lead.

22. A multi-phase alloy consisting essentially of a base constituent consisting essentially of lead and sulphur, the percent by weight of lead being 86.63% to 87.10%, balance substantially all sulphur, having a phase constituting primarily the intermetallic compound lead-sulphide and having another phase constituting primarily excess lead, and no more than of the order of 0.001% by weight of other matter, except for a promoter selected from the group consisting of zirconium, indium, bromine, chlorine, titanium, iodine, tantalum, bismuth, antimony, gallium, columbium, uranium, sodium, potassium, rubidium and silver in an amount effective to modify the conductivity of the base constituent not in excess by weight percent of the lead and sulphur of said promoters as follows: 0.40 zirconium; 0.50 indium; 0.35 bromine; 0.15 chlorine; 0.20 titanium; 0.55 iodine; 0.70 tantalum; 0.30 gallium; 0.40 columbium; 1.0 uranium; 0.20 sodium; 0.30 potassium; 0.70 rubidium; 2.0 silver; and bismuth and antimony not in excess of from 1.0 to 3.0 and from 0.50 to 3.0, respectively, over the aforementioned range of lead.

References Cited in the file of this patent  
or the original patent

55 "Chemical Abstracts," vol. 47, pages 2591(d), 3720(c) and 6246(a). Published by The American Chemical Society, 1953.